

Sept. 13, 1932.

F. M. VENZIE

1,877,209

PLASTER BOARD

Filed April 26, 1930



## UNITED STATES PATENT OFFICE

FREDERICK M. VENZIE, OF PHILADELPHIA, PENNSYLVANIA

## PLASTER BOARD

Application filed April 26, 1930. Serial No. 447,586.

This invention, generally stated, relates to a building structure such as is employed for interior constructions such as walls, partitions, and ceilings and has more especial relation to an improved plaster board such as is calculated to receive a finishing coat of plaster.

Plaster boards of the general type under consideration are of rectangular configuration and are composed of body portion of plaster-like composition sufficiently soft to permit the same being readily cut and nailed to place in the structure being formed. Practice dictates that the composition body, unless of relatively large cross-section, readily breaks; and further, if formed sufficiently thick in cross-section to overcome the fault of ready breakage, is far too bulky for desired purposes in interior constructions. This fault has been partly overcome in the plastering trade by providing a plaster board which is relatively thin in cross-section and enveloping or encasing the same by means of a thin paper covering in order to hold the plaster composition in place. This is an expensive procedure and is not altogether satisfactory for the reason that the plaster board is still subject to more or less ready breakage and may be easily torn apart.

I have discovered that by introducing a suitable reinforce to the body of a relatively thin plaster board I am enabled to so strengthen the plaster board that it is practically impossible to tear the same apart under unusual conditions, and that under normal or ordinary working conditions breakage is reduced to a minimum, and that I may dispense entirely with the paper cover or envelope for strengthening purposes, although under certain conditions where it is deemed necessary or desirable I may employ upon one face of the plaster board a thin sheet of paper properly processed to resist dampness.

The leading object of the present invention is to provide a plaster board of the character stated comprised of a relatively thin and relatively soft body of a plaster-like fire resisting composition having embedded therein one or more sheets of coarse mesh reinforcing mate-

rial as burlap or other woven material which may be readily cut.

A further object of the present invention is to provide a plaster board of the character stated having embedded therein one or more sheets of coarsely woven material the mesh of which permits the relatively soft body penetrating the sheet or sheets of woven material to provide in effect a unitary or integral structure requiring in fact a cutting process to destroy its efficiency.

A further object of the present invention is to provide a plaster board of the character stated and reinforced as described having that face thereof adapted to receive a coating of plaster scored in order that an efficient bond may be secured between the plaster-like body of the plaster board and the coating of plaster.

With these and other objects in view, as will hereinafter appear, the invention consists of the novel construction hereinafter described and finally claimed.

The nature, characteristic features and scope of the invention will be more fully understood from the following description taken in connection with the accompanying drawings forming part hereof, and in which:

Fig. 1 is a perspective view of a plaster board embodying the invention and illustrating the same as having two plane surfaces;

Fig. 2 is a similar view of the same but having a somewhat modified form of reinforcement;

Fig. 3 is a view similar to Fig. 1, but illustrating the plaster board as having a roughened surface;

Fig. 4 is a fragmentary view in section of the plaster board as having a plane surface, a roughened surface, and a reinforcement similar to that shown in Fig. 2;

Fig. 5 is a view similar to Fig. 4 but showing a paper covering applied to the unroughened surfaces;

Fig. 6 is a view similar to Fig. 5 but showing the paper covering as having a coating of moisture resisting material applied thereto; and

Fig. 7 is a top or plan view of a plaster board with its paper cover broken away.

For the purpose of illustrating my invention I have shown in the accompanying drawing several forms thereof which are at present preferred by me, since the same have been found in practice to give satisfactory and reliable results, although it is to be understood that the various instrumentalities of which my invention consists can be variously arranged and organized and that my invention is not limited to the precise arrangement and organization of the instrumentalities as herein shown and described.

In the manufacture of my novel plaster board which is of rectangular form, relatively thin, and relatively soft, I form the body 10 of a plaster-like composition which may be of any desired combination of materials to provide a fire-resisting structure. In practice good results have been obtained by employing plaster, cork, and silicate of soda in dry powdery form, and in suitable proportions, to which is added other desired ingredients and sufficient water to render the mixture plastic to be molded to desired shape. Such a plaster board is very light in weight, is porous, but is readily breakable because it is relatively dry and powder-like. To strengthen and reinforce such body 10, I embed therein, at the time of molding, a sheet or sheets of loosely woven burlap designated 11. I prefer to use burlap because it is very cheap and has a very coarse mesh, so that the plaster composition may readily pass between the mesh and in effect form an integral structure which makes it relatively difficult to tear or break the body 10 unless the same is cut. While I prefer to use burlap because it is cheap and of coarse mesh, obviously other reinforcing material which is woven in character may be employed, as for instance: fish net, strong grades of linen or cotton mosquito netting, and wire netting.

Referring now to Fig. 1, the plaster board 10 which is relatively fire-proof in make-up is provided with plane surfaces 12 and has embedded in the body of the plaster board a single sheet of loosely woven burlap.

The construction of parts shown in Fig. 2 is similar in all respects to that shown in Fig. 1 except that two sheets of loosely woven burlap, spaced apart, are employed.

The construction shown in Fig. 3 is similar in all respects to the showing made in Fig. 1 with the exception that one surface of the plaster board is roughened to more readily accept a coat of plaster. The specific form of roughened surface shown comprises a corrugated-like surface 13 which may be obtained by scoring the surface of the plaster board.

The showing made in Fig. 4 is similar in all respects to the construction shown in Fig. 3 with the exception that two sheets of burlap reinforcement are employed instead of the

single sheet of burlap reinforcement shown in Fig. 3.

The showing made in Fig. 5 is similar in all respects to the construction shown in Fig. 4 with the exception that a thin sheet of paper 14 is applied to one face and two sides of the plaster board.

The showing made in Fig. 6 is similar in all respects to the construction shown in Fig. 5 with the exception that the sheet of paper 14 may have applied thereto a coating 15 of any desired damp-proofing material, as asphaltum paint.

I have described a number of different forms in which my plaster board may be manufactured, all of said constructions, however, embodying a plaster board of more or less fragile material reinforced by one or more sheets of loosely woven material, as burlap. In some instances it is desirable to have plane surfaces for the plaster board, and in other cases it is desirable to have the same roughened to more readily accept a coating of plaster. In some instances it may also be desirable to add to the plaster board a paper covering to resist dampness and moisture.

A construction such as is above described is light, strong, and durable and forms a plaster board which is very difficult to break or tear apart, but which may be readily cut or sawed. Not only is my plaster board possessed of the above advantages, but it is also sound resisting in character.

In the above described plaster board I prefer first to form a plaster board of plaster of Paris in the proportion of about 80% in bulk and add about 10% of powdered cork and about 10% of asbestos. When mixing the above ingredients with water I add about 20% of silicate of soda to render the finished plaster board impervious to water.

The plaster board above described is of a cross-section which does not exceed one half inch in thickness and it is often desirable to make the plaster board so that it measures in thickness as low as  $\frac{3}{16}$  of an inch, as where, for instance, the plaster board is employed for backing other softer material in which designs are required.

Referring now to Fig. 7, I show a plaster board body 16 which may be reinforced or not as desired and has applied to a face thereof a thin sheet of paper 17 which is provided with a plurality of cuts or scores 18 arranged in staggered relation. When a sheet of paper is glued or cemented to a body of plaster like make-up the moisture resulting has the tendency to warp the body, which is undesirable. I have discovered that by cutting the paper therethrough, as shown in Fig. 7, shrinkage of the paper is taken up by the cuts 18 and thereby prevents the paper pulling the body out of place or warping the same. By staggering the cuts 18 as shown

the paper is prevented from shrinking in a direct line.

I am aware that the invention may be embodied in other specific forms without departing from the spirit or essential attributes thereof, and I therefore desire the present embodiment to be considered in all respects as illustrative and not restrictive, reference being had to the appended claim rather than to the foregoing description to indicate the scope of the invention.

What I claim is:

A plaster board of the character stated comprising a rectangular shaped, relatively thin body of plaster composition of dry powdery consistency the particles thereof being held together by a reinforcing sheet of fibrous material only composed of loosely woven wefts and warps which material may be readily severed, said sheet being embedded in said body throughout its extent considered in length and breadth, the inner face of said body having a plane surface, and the outer face of said body being corrugated in parallelism with the wefts of said sheet of fibrous material to provide a roughened surface more readily to accept a coat of plaster, and a thin sheet of paper possessing moisture resisting properties applied to the inner plane face of said body, the combined body, sheet of fibrous material, and paper forming a unitary structure.

FREDERICK M. VENZIE.

35

40

45

50

55

60

65